

## 1

2,982,649

## PRODUCTION OF COLORED PHOTOGRAPHIC IMAGES

Bernard Hippoliet Tavernier and Marcel Léon Desmit, Antwerp, and Arthur Henri De Cat, Mortsel-Antwerp, Belgium, assignors to Gevaert Photo-Producten N.V., Mortsel, Belgium, a Belgian company

No Drawing. Filed Mar. 10, 1958, Ser. No. 719,994

6 Claims. (Cl. 96—55)

The present invention relates to a process for the manufacture of colored photographic images by color development in the presence of a color coupler, to photographic developers which contain such color coupler and to photographic images obtained according to this process.

It is known to obtain a colored photographic image by developing a reducible silver salt image in the presence of a color coupler, i.e. a compound which during development couples with the oxidation product of the developing agent and forms a dyestuff which precipitates onto the developed silver grains.

Yellow colored images are usually obtained by development in the presence of compounds which contain an active methylene group, particularly acylacetanilide derivatives.

Among the acylacetanilide derivatives, those which are substituted in their anilide part by a sulphonamide group are known to have the property of being highly soluble in the developer whilst the resulting dyestuffs nevertheless have no tendency to bleed out.

It is an object of the present invention to provide a new process of color development, more particularly in the presence of a color coupler, which is more reactive than the known sulphonamido substituted acylacetanilides. It is another object of the present invention to provide a new color developer containing such a color coupler. It is a further object of the present invention to provide new colored photographic images obtained by such process. Still further objects will appear from the description hereinafter.

According to the present invention, these objects are accomplished by developing a reducible silver salt image with an aromatic amino developing agent in the presence of an aliphatic, aromatic or heterocyclic acyl acetylarylide, the arylide part of which is substituted in 2-position by an alkoxy group and in 5-position by an alkyl or aryl sulphonamide group.

These compounds may be obtained as follows: 1 mol of a 3-acetamino-4-alkoxy-benzene sulphochloride, for instance the 4-methoxy compound described by K. Child, J. Chem. Soc. (1932), 715/720, is added at 40—50° C. to 2 mols of a primary amine dissolved in dioxane. After refluxing for ninety minutes the precipitate obtained on cooling is sucked off, washed with water and recrystallized.

In this way the following can be prepared:

3 - acetamino - 4 - methoxy - benzene - n - butyl - sulphonamide, melting at 114—115° C.,

3 - acetamino - 4 - methoxy - benzene - phenyl - sulphonamide, melting at 198—200° C.,

3 - acetamino - 4 - methoxy - benzene - p - methoxyphenyl-sulphonamide, melting at 162—164° C.

These compounds are mixed with 10% of a concentrated solution of hydrogen chloride in methanol. The mixture is refluxed and next neutralized with ammonium hydroxide. The precipitate thus obtained is sucked off and washed with water.

## 2

In this way the following can be obtained:

3-amino-4-methoxy-n-butyl-sulphonamide, melting at 99—100° C.,

3-amino-4-methoxy-phenyl-sulphonamide, melting at 139—140° C.,

3 - amino - 4 - methoxy - p - methoxyphenyl - sulphonamide, melting at 135—136° C.

These compounds are refluxed with an excess of beta-keto ester. The precipitate obtained on cooling is sucked off, washed with a diluted acid and recrystallized until white crystals are obtained.

In this way the following can be prepared:

(1) 3(benzoyl - acetyl - amino) - 4 - methoxy - benzene-n-butyl-sulphonamide, melting at 95—97° C.,

(2) 3(benzoyl - acetyl - amino) - 4 - methoxy - benzene-p-methoxyphenyl-sulphonamide, melting at 179—180° C.,

(3) 3(benzoyl - acetyl - amino) - 4 - methoxy - benzene-phenyl-sulphonamide, melting at 160—161° C.,

(4) 3(acetyl - acetyl - amino) - 4 - methoxy - benzene-phenyl-sulphonamide, melting at 196—197° C.,

(5) 3(alpha - thenoyl - acetyl - amino) - 4 - methoxybenzene-phenyl-sulphonamide, melting at 200—202° C.,

(6) 3(p - methoxy - benzoyl - acetyl - amino) - 4 - methoxy-benzene-phenyl-sulphonamide, melting at 194° C.

The presence during color development of color couplers according to the present invention may arise from adding to the developer a compound which differs from the color coupler only because in the active CH<sub>2</sub>-group one or two hydrogen atoms are replaced by a group capable of splitting off either before development occurs by the action of the alkali in the developing solution or during the color-development.

The aromatic amino compounds, which according to our invention are used as developing agents, comprise mono-, di- and tri-amino aryl compounds, particularly N:N-dialkyl-paraphenylene diamines and derivatives such as N:N-dialkyl-N'-sulphonethyl-para-phenylene diamines. As mono-amino developers amino-phenols, amino-cresols and their halogen derivatives, and also amino-naphthols may be mentioned.

The following example serves to illustrate the invention without, however, limiting the scope thereof.

An exposed photographic film strip coated with a silver halide emulsion layer is developed in a bath of the following composition:

|    |                                                     |     |
|----|-----------------------------------------------------|-----|
| 50 | Solution A:                                         | G.  |
|    | Sodium hexa-meta-phosphate                          | 1   |
|    | Sodium sulphite (anhydrous)                         | 3   |
|    | N:N-diethyl-p-phenylene-diaminehydrochloride        | 3   |
| 55 | Sodium sulphate (anhydrous)                         | 40  |
|    | Sodium carbonate (anhydrous)                        | 35  |
|    | Potassium bromide                                   | 1.5 |
|    | Water to 900 cm. <sup>3</sup>                       |     |
| 60 | Solution B:                                         | G.  |
|    | Sodium hydroxide                                    | 1.5 |
|    | One of the couplers 1—6 prepared as described above | 1   |
|    | Water to 50 cm. <sup>3</sup>                        |     |

Before use, solution B is added to solution A and water is added to the resulting solution to 1,000 cm.<sup>3</sup>. The developed image is rinsed for thirty minutes and the silver is bleached in the following bath:

|    |                                 |    |
|----|---------------------------------|----|
| 70 | Potassium ferricyanide          | G. |
|    | Potassium bromide               | 3  |
|    | Water to 1,000 cm. <sup>3</sup> |    |

The image is rinsed again for ten minutes and then fixed for twenty minutes in the following bath:

Sodium thiosulphate----- 250 g.  
Water to----- 1,000 cm.<sup>3</sup>.  
and again rinsed for thirty minutes.

A yellow image is obtained.

We claim:

1. Process for producing a colored photographic image by developing a reducible silver salt image with p-diethylamino-aniline hydrochloride as an aromatic amino developing agent in the presence of an acylacetanilide coupler, whereby said coupler is 3(benzoyl-acetyl-amino)-4-methoxy-benzene-phenyl-sulphonamide. 10

2. Photographic color developer containing p-diethylamino-aniline hydrochloride as an amino aromatic developing agent and a color coupler, whereby said coupler is 3(benzoyl-acetyl-amino)-4-methoxy-benzene-phenyl-sulphonamide. 15

3. Photographic color developer containing p-diethylamino-aniline hydrochloride as an amino aromatic developing agent and a color coupler, whereby said coupler is 3(acetyl-acetyl-amino)-4-methoxy-benzene-phenyl-sulphonamide. 20

4. Photographic color developer containing p-diethylamino-aniline hydrochloride as an amino aromatic developing agent and a color coupler, whereby said coupler is 3(thenoyl-acetyl-amino) - 4-methoxy-benzene-phenyl-sulphonamide. 25

5. Process for producing a colored photographic image 30

by developing a reducible silver salt image with p-diethylamino-aniline hydrochloride as an aromatic amino developing agent in the presence of an acylacetanilide coupler selected from the group consisting of 3(benzoyl-acetyl-amino - 4 - methoxy-benzene-n-butyl-sulphonamide, 3-(benzoyl-acetyl-amino)-4 - methoxy-benzene-phenyl-sulphonamide, 3-(benzoyl-acetyl-amino)-4-methoxy-benzene-phenyl-sulphonamide, 3(acetyl-acetyl-amino)-4-methoxy-benzene-phenyl-sulphonamide, and 3(thenoyl-acetyl-amino)-4-methoxy-benzene-phenyl-sulphonamide.

6. Photographic color developer containing p-diethylamino-aniline hydrochloride as an aromatic amino developing agent and an acylacetanilide coupler selected from the group consisting of 3(benzoyl-acetyl-amino)-4-methoxy-benzene-n-butyl-sulphonamide, 3(benzoyl-acetyl-amino)-4-methoxy-benzene-phenyl-sulphonamide, 3(thenoyl-acetyl-amino)-4-methoxy-benzene-phenyl-sulphonamide, and 3(acetyl-acetyl-amino)-4-methoxy-benzene-phenyl-sulphonamide.

#### References Cited in the file of this patent

#### UNITED STATES PATENTS

|           |                    |               |
|-----------|--------------------|---------------|
| 2,271,238 | Vittum et al.      | Jan. 27, 1942 |
| 2,350,138 | Weissberger        | May 30, 1944  |
| 2,407,210 | Weissberger et al. | Sept. 3, 1946 |
| 2,596,755 | Young et al.       | May 13, 1952  |
| 2,694,718 | Salminen et al.    | Nov. 16, 1954 |